

## UNITED STATES PATENT OFFICE

2,226,079

## DENTAL ALLOY

Jakob Spanner, Neu-Isenburg, Germany, assignor,  
by mesne assignments, to Chemical Marketing  
Company Inc., New York, N. Y.

No Drawing. Application May 11, 1938, Serial No.  
207,383. In Germany May 12, 1937

## 1 Claim. (Cl. 75—172)

Objects of my invention are dental alloys which are particularly suited for casting and soldering purposes.

The ordinary alloys with a low melting point such as are used for instance for soldering of dental prostheses consist chiefly of precious metals which may contain in some cases relatively small additions of suitable non-precious metals. The dental solders which are most commonly in use are for instance gold-, silver-, copper-alloys and palladium-silver-alloys with addition of such metals as zinc and cadmium.

The objects of this invention are alloys with relatively small contents of precious metals which are particularly suitable for the purposes of casting and soldering artificial dentures.

I have found that this purpose is served in an excellent manner by the application of such alloys as contain palladium as precious metal and metals of the iron group as non-precious metals, the latter metals being used either singly or in combination of several of them.

A dental alloy in accordance with my invention which is particularly useful consists for instance of about 20-60 parts, in preference of about 30-45 parts by weight of palladium, the rest being iron, nickel, cobalt either alone or in combination of two or more of the latter.

Alloys of the described kind do not tarnish and are very resistant against the attack of aggressive agents such as occur in the mouth. They further excel by the fact that they can be very easily cast, they can easily be worked upon and are especially suitable for soldering parts of metals which have a high melting point for instance such which consist of non-tarnishing steel such as are for instance known by the trade as V.A-steel or cobalt-chromium-tungsten-alloys such as are used for dental prostheses.

The alloys may contain such additional metals

as are customary for casting alloys and solders. Such additions are for instance copper, silver, zinc, cadmium, manganese, chromium, tin either singly or a mixture of two or more of them in similar quantities, for instance up to 10 or even up to 15%. These metals have the effect of lowering the melting point of the alloys.

The following are a number of examples which show compositions of alloys according to my invention:

## Example 1

|    | Parts<br>by weight |    |
|----|--------------------|----|
| Pd | 45.1               | 15 |
| Fe | 54.0               |    |
| Mn | 0.9                |    |

## Example 2

|    |      |    |
|----|------|----|
| Pd | 36.0 | 20 |
| Ni | 58.0 |    |
| Cu | 4.0  |    |
| Mn | 0.5  |    |
| Zn | 1.5  | 25 |

## Example 3

|    | Per cent<br>by weight |    |
|----|-----------------------|----|
| Pd | 25-40                 |    |
| Cr | 4-15                  | 30 |

Rest Ni and small quantities of Mg.

What I claim is:

A dental alloy which consists of 20-60 percent of palladium, 4-15 percent of chromium and the remainder substantially all iron, said dental alloy being characterized in being easily cast, tarnish resistant, resistant against the attack of aggressive agents occurring in the mouth, and suitable for soldering.

JAKOB SPANNER. 40